

Nov. 29, 1927.

1,650,987

J. HOLTHAUS

PROCESS OF CENTRIFUGALLY MOLDING METALS

Filed Aug. 18, 1925



Inventor:

Dr. Johann Holthaus

per *Holthaus*

Attorney.

## UNITED STATES PATENT OFFICE.

JOHANN HOLTHAUS, OF GELSENKIRCHEN, GERMANY.

## PROCESS OF CENTRIFUGALLY MOLDING METALS.

Application filed August 18, 1925, Serial No. 50,960, and in Germany August 26, 1924.

In the process of centrifugally casting tubes and other hollow bodies, where the liquid metal is fed through a spout into the rotating mold, the spout being gradually withdrawn from the mold, or the latter being moved longitudinally relatively to the fixed spout, the stream of metal discharged from the spout is coiled on the inner surface of the mold, and the usual method is to produce at first the thicker or butt end of the hollow body, in the case of producing tubes, the socket end, then the cylindrical part, and finally the spigot or cylindrical end. In the case of metals with high coefficients of shrinkage, for example steel, and metals which quickly harden after the casting, or in the mold, it is found, that tubes and the like so cast are liable to crack transversely, sometimes so seriously as to break apart. This is largely due to the fact that the enlarged or butt end of the hollow body cannot yield sufficiently to counteract the deleterious effects of shrinkage.

According to this invention this defect is overcome, when metals of the kind referred to are used, by first casting the cylindrical or spigot end, then the intermediate smooth or cylindrical part, and then the enlarged or socket end. With this method the portions first cast are able freely to yield in the longitudinal direction while the butt end is still in the transition stage between the liquid and solid states, and risk of cracking is thus eliminated or at least greatly reduced.

I am aware that it has been heretofore proposed to centrifugally mold pipes in such manner that the long central portion of the pipe is first molded and then the spigot end and the socket end are formed simultane-

ously so that the long pipe part can yield during the shrinking process. In this known arrangement, however, two casting spouts are required to supply the metal to the center of the mold, but in accordance with the present invention the same effect is produced by means of a single spout so that complicated and expensive means for moving and changing the two casting spouts are entirely eliminated.

In order that this invention may be more clearly understood and readily carried into effect, a suitable form of apparatus is illustrated on the accompanying drawing wherein *a* is a mold mounted on supporting wheels *b* and adapted to move during the casting operation in the direction of the arrow *R*. The spout *c* extends through the end *e* of the mold and the metal is supplied to the spout from the ladle *d*. The drawing shows the position at the commencement of the casting operation, and as soon as the metal begins to flow into the mold the latter is moved in the direction so that the spigot end of the pipe is first formed and the socket end is formed only at the end of the operation.

What I claim as my invention and desire to secure by Letters Patent of the United States is:—

The process of centrifugally casting hollow bodies in a centrifugal casting machine with only one relatively displaceable spout, which consists in first casting the spigot end, then the intermediate portion, and finally the socket end.

In witness whereof I have signed this specification.

DR. JOHANN HOLTHAUS.